

# UNITED STATES PATENT OFFICE.

GEORGE ROSS AND STEPHEN F. DEAL, OF KANSAS CITY, MISSOURI

## PROCESS OF FACING ROADWAYS, STREETS, AND WALKS.

No. 838,551.

Specification of Letters Patent.

Patented Oct. 16, 1906.

Application filed January 12, 1906. Serial No. 295,811.

*To all whom it may concern:*

Be it known that we, GEORGE ROSS and STEPHEN F. DEAL, citizens of the United States, residing at Kansas City, in the county of Jackson and the State of Missouri, have invented certain new and useful Improvements in Processes of Facing Roadways, Streets, and Walks, of which the following is a specification.

10 This invention relates to a process for making roadways, street-pavements, and sidewalks, and has for its object to provide a roadway, pavement, or sidewalk with a facing practically impervious to water and of durable construction.

15 A further object is to evolve a process by which roadways and the like can be provided with a facing of any required depth, of the character named, expeditiously and at comparatively low cost.

20 In carrying out the invention we first plow, harrow, or otherwise loosen and pulverize the ground to a suitable depth, the roadway at the same time being also brought to the desired grade if a change of grade is necessary or desirable.

25 A liquid or plastic binder, preferably the former, is produced by heating and mixing asphaltum with oil of any suitable character, preferably crude or unrefined oil, and then this binder is deposited in any suitable manner upon the prepared ground, the distribution of the binder being made as even as possible in order to avoid undue waste thereof.

30 This binder is mixed with the pulverized earth, and then the road is rolled or tamped to the required density, so as to produce a comparatively smooth and even surface. A facing thus produced is tough and tenacious and will not break up or crumble and result in loss of material like an asphalt pavement, because the oil or equivalent substance prevents water from soaking into the roadway.

35 Furthermore, its tough, tenacious, and homogeneous properties give it such elasticity that it will yield under the passage of a heavy vehicle over it without chipping or crumbling, and as a result no dust will gather on its surface other than that blown there.

40 The road-facing above described will be employed preferably on country roads.

45 For city streets it is preferable to first loosen and pulverize the earth as explained. The mixture of asphaltum and oil is then deposited thereon and harrowed or otherwise intimately mixed therewith. Then a layer of

5 granular substance—for instance, granite chips, Joplin, or native grit—is deposited on the earth as thus prepared. Then a second mixture of asphaltum and oil is deposited on the layer of granular substance, and then the grit, with the second mixture of asphaltum and oil, is so stirred as to make it a part of the upper surface of the earth prepared as aforesaid. The prepared earth is then thoroughly 65 tamped or rolled, or both tamped and rolled, to provide a smooth and even surface.

60 Where it is desirable to produce a road-facing similar to the common asphalt pavement, a suitable quantity of sulfur may be 70 mixed with the asphaltum and oil as a hardener.

75 A roadway, street-pavement, or walk treated according to the process described will obviously not only prevent water from seeping down into the facing, but will prevent moisture below from ascending through said facing.

80 The roadway, street, or walk prepared as described not only possesses the features of advantage described, but is easy on the feet of the animals traversing it, and comparatively noiseless.

85 From the above description it will be apparent that we have evolved a process for producing facings for roadways and the like which is durable, practically impervious to water, and possesses the other desirable features named herein.

Having thus described the invention, 90 what we claim as new, and desire to secure by Letters Patent, is—

1. The process of facing roadways and the like, consisting in loosening and pulverizing the earth to a suitable depth, depositing a binder therein impervious to water and having tough and tenacious properties, and then compacting the mass of loose earth containing the binder in any suitable manner.

2. The process of facing roadways and the like, consisting in loosening and pulverizing the earth to a suitable depth, depositing a binder therein impervious to water and having tough and tenacious properties, and then compacting the mass of loose earth containing the binder by running a roller over it.

3. The process of facing roadways and the like consisting in loosening and pulverizing the earth to a suitable depth, depositing a binder therein impervious to water and having tough and tenacious properties, then in depositing a layer of granular material on the

earth thus prepared, then in making a second deposit of said binder on said layer of granular material, then in mixing said second deposit of the binder and said granular material with the upper portion of the mass of earth mixed with the first deposit of the binder, and finally in compacting the mass of loose earth containing the first deposit of the binder with the granular material and the second deposit of the binder.

4. The process of facing roadways and the like consisting in loosening and pulverizing the earth to a suitable depth, depositing a binder therein which is impervious to water and has tough, tenacious and hardening properties, and then compressing the entire mass of loosened earth thus treated down upon the solid earth beneath.

5. The process of facing roadways and the like consisting in loosening and pulverizing the earth to a suitable depth, depositing a binder therein which is impervious to water and has tough, tenacious and hardening properties, and then compressing the en-

tire mass of loosened earth thus treated 25 down upon the solid earth beneath by running a roller over it.

6. The process of facing roadways and the like, consisting of loosening and pulverizing the earth to a suitable depth, depositing a 30 binder therein consisting of asphaltum and oil in a liquid state, and then compacting the mass of earth containing the binder.

7. The process of facing roadways and the like, consisting in loosening and pulverizing 35 the earth to a suitable depth depositing a binder of mixed melted asphaltum and oil thereon, in mixing granular material, with the earth thus treated, and finally in compacting the mass of loose earth containing 40 the binder and granular material.

In testimony whereof we affix our signatures in the presence of two witnesses.

GEORGE ROSS.  
STEPHEN F. DEAL.

Witnesses:

E. M. METCALF,  
W. M. RYNERSON.